

Oct. 20, 1942.

B. K. GREEN

2,299,694

MANIFOLDING MATERIAL

Filed March 9, 1940



Barrett K. Green  
Inventor

By *Karl Bensd*  
His Attorney

Patented Oct. 20, 1942

2,299,694

# UNITED STATES PATENT OFFICE

2,299,694

## MANIFOLDING MATERIAL

Barrett K. Green, Dayton, Ohio, assignor to The National Cash Register Company, Dayton, Ohio, a corporation of Maryland

Application March 9, 1940, Serial No. 323,155

19 Claims. (CL 106—236)

This invention relates to manifold paper and more particularly to manifold paper that is proof against smudging.

Most manifold paper now in use has a coating consisting of a waxy solid, containing coloring matter, which is transferred to the surface of an underlying sheet by impact or pressure. The coating is easily rubbed off on the fingers or onto an underlying sheet by ordinary handling, causing the fingers or the underlying sheet to be smudged. The underlying sheet, after having the colored coating transferred to its surface, is subject to smudging, if rubbed, and in addition is subject to erasure, because the solid transferred material does not enter into the fibre of the paper but merely adheres to the surface.

It is the principal object of this invention to provide a smudge-proof manifold sheet.

A further object of the invention is to provide a manifold sheet having a coating of fluid transfer material which is releasable therefrom, by impact or pressure, so as to be transferred to and to penetrate the underlying sheet.

A further object of the invention is to provide a manifold sheet having a coating that is normally dry on its surface and smudge-proof in ordinary manipulations.

Another object of the invention is to provide a manifold sheet having a solid coating containing fluid inclusions of coloring matter.

Another object of the invention is to provide a manifold paper having a color-producing transfer coating, the exposed surface of which is free of coloring matter.

With these and incidental objects in view, the invention includes certain novel features, the essential elements of which are set forth in appended claims and a preferred form or embodiment of which is hereinafter described with reference to the drawing which accompanies and forms a part of this specification.

The drawing represents a cross-section of a manifold sheet made in accordance with this disclosure, showing, in diagrammatic and enlarged form, the fluid inclusions in the coating.

### GENERAL DESCRIPTION

The manifold sheet comprises a base sheet 28 of paper, tissue, or other web-like substance used for printing or writing, upon one surface of which sheet is deposited a coating comprising a rupturable semi-soft colorless solid 21 having profusely dispersed therein discrete fluid-containing cells 22 so small as to be invisible to the unaided eye. The fluid in cells 22 is either an

ink, stain, or other coloring matter, or has suspended or dissolved therein ink, pigment, stain, or other coloring matter, or contains coloring matter in an emulsion. Upon impact or pressure against the manifold sheet by a printing member or a writing member, the solid coating is locally ruptured through to its surface so that the fluid inclusions will be released at the place of impact, to be locally absorbed by the underlying transfer sheet according to the contours 5 of the type face of the printing member or according to the contours traced by the writing member. Because the fluid-containing cells 22, whose contents are so transferred, are individually small enough to be invisible to the unaided eye, they are supplied in the solid in profuse quantities so as to cause the transfer thereof to appear as a continuous visible mark, in a mosaic manner. This transferred substance, being fluid, acts as fluid ink acts, penetrating the fibres of the underlying sheet and drying thereon by absorption. For this reason, erasures cannot be made on the underlying sheet without seriously eroding its fibres, and the drying of the fluid leaves the underlying sheet smudge-proof.

In making the coating, the ultimate continuous and solid phase of the coating is dissolved in a drying liquid to form a solution into which the ultimate fluid discontinuous inclusions of the coatings are emulsified. The emulsion is then coated on the manifold sheet and the drying liquid, evaporating, leaves the solid coating with fluid discrete inclusions dispersed profusely therethrough. In selecting the ingredients of the coating, the solid phase must be impervious to the fluid inclusions, chemically inactive with them, easily rupturable by ordinary printing and writing pressures, and subject to having introduced therein plasticizers and hygroscopic control substances to meet special conditions of use and special weather conditions. The dispersed fluid inclusions phase must not be affected chemically by or absorbed by the solid phase.

The invention is best embodied by the use of 45 finely divided carbon black suspended in a fluid for the fluid inclusion phase, which is then emulsified in a temporarily fluid continuous phase comprising semi-solid materials dissolved in a drying liquid. The semi-solid materials of the 50 continuous phase are selected for their properties of being colorless, pliable under pressures of ordinary manipulation, but brittle under rapidly applied pressures and rupturable by heavy pressures as encountered in the printing arts. The drying liquid is selected so that, after being ap-

plied to the paper, it dries quickly, leaving the solid phase with the fluid inclusions dispersed therein. The following formula is given for the proportions by weight of the continuous and dispersed phases of such an emulsion:

*Solid coating or continuous phase 75% by weight*

Per cent by weight

Gum dammar ..... 50  
Toluene ..... 50

*Fluid inclusions or dispersed phase 25% by weight*

Per cent by weight

Glycerine ..... 80  
Polyethylene glycol ..... 14  
Carbon black ..... 6

The dispersed phase of the emulsion may be made as fine as desired, a particle size of .1 millimeter being sufficiently small to cause a continuous appearance to the unaided eye in the transfer providing the inclusions are supplied in profuse quantities so as to cause them to be about the same distance apart as their diameter. Ordinary emulsifying procedure may be used.

After the application of the above-mentioned emulsion to the manifold sheet, the toluene evaporates, the then solid gum dammar acting to isolate the dispersed fluid inclusions from one another and protecting them from the evaporating and drying effect of the air.

With the proportions given, the impact of the ordinary stroke of a printing member or the pressure of a writing member is sufficient to cause a rupture of the coating, yet the coating is smudge-proof against ordinary handling.

Because the carbon black is finely divided, it is carried by the suspending fluid of the dispersed phase, as the coating is ruptured, into the fibre of the underlying sheet, as is the pigment in ordinary ink, making the transferred coloring matter on the underlying sheet smudge-proof and resistant to erasure.

Dyes may be used in place of such pigments as the above-described carbon black. For an example of a dye coloring matter the following formula is given for the dispersed phase of the emulsion coating in place of that given for the carbon black type of coating:

*Dispersed phase 25%*

Per cent

Glycerine ..... 97  
Malachite green ..... 3

It is not intended that the formulas given shall limit the invention, as the principle involved is applicable to any coating containing minute and profuse inclusions of fluids containing coloring matter, which fluids are released for transfer by locally rupturing the surface of the coating.

While the form of the invention herein shown and described is admirably adapted to fulfill the objects primarily stated, it is to be understood that it is not intended to confine the invention to the one form or embodiment herein disclosed, for it is susceptible of embodiment in various forms all coming within the scope of the claims which follow.

What is claimed is:

1. A manifold sheet comprising a base sheet and a coating on the base sheet having discrete fluid inclusions of coloring matter profusely dispersed therein.

2. A manifold sheet comprising a base sheet and a coating on the base sheet having pigment-

bearing discrete fluid inclusions profusely dispersed therein.

3. A manifold sheet covered profusely with minute, rupturable, liquid-containing cells, the liquid released from said cells by rupture being able to visibly affect a second sheet if in contact therewith.

4. In combination, a sheet of paper, and a plastic coating on said sheet, said plastic coating containing discrete inclusions of carbon black suspended in a liquid.

5. A manifold sheet for transferring printing materials to another sheet by impact, comprising a profuse number of liquid staining discrete inclusions imbedded in a rupturable coating on the manifold sheet.

6. A non-smudging manifold sheet having a coating consisting of a profuse number of minute discrete inclusions of liquid printing ink in a locally rupturable plastic solid medium.

7. A liquid composition for coating paper, consisting of a solution of gum dammar in toluene having emulsified therein a polyhydric alcohol printing solution.

8. An emulsion for coating paper, consisting of a solution of gum dammar and toluene as a continuous phase, and carbon black suspended in a glycerol solution as a discontinuous phase.

9. In combination, an impression sheet; a transfer sheet; and, on said transfer sheet, an intervening film of solid substance having dispersed therein discrete liquid inclusions of coloring matter, said liquid in said inclusions being transferable to the impression sheet upon rupture of the solid substance in conformance with any impression made on the transfer sheet.

10. An emulsion for coating paper having a continuous phase which is a solution of

Per cent by weight  
Toluene ..... 50  
Gum dammar ..... 50  
taken three parts, and the discontinuous phase of which is

Per cent by weight  
Glycerine ..... 80  
Polyethylene glycol ..... 14  
Carbon black, or other pigment ..... 6  
taken one part, and emulsified so that the discontinuous phase is of a particle size invisible to the unaided eye.

11. An emulsion for coating paper having a continuous phase which is a solution of

Per cent by weight  
Toluene ..... 50  
Gum dammar ..... 50  
taken three parts, and the discontinuous phase of which is

Per cent by weight  
Glycerine ..... 97  
Malachite green ..... 3  
taken one part.

12. An emulsion for coating paper having a continuous phase which is a solution of

Per cent by weight  
Toluene ..... 50  
Gum dammar ..... 50  
taken three parts, and the discontinuous phase of which is

Per cent by weight  
Glycerine ..... 97  
A dye insoluble in toluene ..... 3  
taken one part.

13. A manifolding paper having a colorless coating thereon containing a profuse number of fluid cell inclusions of coloring matter, said inclusions being so small as to be invisible to the unaided eye, the said coating holding said fluid of the cells incased against external contact under ordinary handling but, by the cells being ruptured, releasing the fluid of the cells at the point of a printing impact so that the fluid may be transferred to an underlying sheet.

14. A manifold sheet having coated thereon a semi-solid non-transferable substance rupturable by printing pressures, which substance contains discrete fluid inclusions of coloring matter which are transferable to an underlying sheet by a rupture of the said semi-solid substance.

15. A manifold sheet having a non-transferable coating thereon which is smudge-proof to ordinary handling but which contains dispersed therein cells of coloring matter which may be freed to effect a transfer by pressures which rupture the coating.

16. A non-smudging manifold sheet having coated thereon a semi-solid non-transferable substance containing discrete fluid inclusions of

coloring matter in a polyhydric alcohol solution, which fluid is retained against external contact and evaporation by the semi-solid substance until released therefrom by rupture of the semi-solid substance.

17. A non-smudging manifold sheet having thereon a gum dammar coating containing a dispersion of discrete liquid inclusions of coloring matter in a polyhydric alcohol solution.

18. A manifolding sheet having a coating containing a discontinuous phase of minute liquid inclusions of coloring matter in a glycerol solution encased in a non-transferable semi-rigid continuous phase of gum dammar, said continuous phase protecting the discontinuous phase from external contact and evaporation until the continuous phase is ruptured to free the liquid inclusions.

19. A manifold sheet having a coating of locally rupturable gum dammar, which coating has therein a profusion of minute discrete liquid-retaining cells containing coloring matter in a glycerol solution, said cells releasing the liquid therein when the coating adjacent thereto is ruptured.

BARRETT K. GREEN.